

L. C. BASSFORD,  
INSULATING SUBSTANCE,  
APPLICATION FILED MAR. 22, 1913.

1,172,926.

Patented Feb. 22, 1916.



Witnesses:

Harry S. Gaither  
Wm. M. Ford

by

Lowell C. Bassford  
Banning & Banning  
Attn.

# UNITED STATES PATENT OFFICE.

LOWELL C. BASSFORD, OF CHICAGO, ILLINOIS, ASSIGNOR TO GENERAL RAILWAY SUPPLY CO., OF CHICAGO, ILLINOIS, A CORPORATION OF ILLINOIS.

## INSULATING SUBSTANCE.

1,172,926.

Specification of Letters Patent. Patented Feb. 22, 1916.

Application filed March 22, 1913. Serial No. 756,260.

To all whom it may concern:

Be it known that I, LOWELL C. BASSFORD, a citizen of the United States, residing at Chicago, in the county of Cook and State of Illinois, have invented certain new and useful Improvements in Insulating Substances, of which the following is a specification.

The present invention relates to an insulating compound more particularly and especially adapted for use in wall constructions, as for instance the walls of sleeping cars etc., for the purpose of preventing the ingress of heat, cold or dampness through the walls and into the interior of the car, and also for the purpose of conserving the heat within the car during cold weather.

The objects of the present invention are to produce a substance for the purpose specified which will be cheap and simple of manufacture and production; which will possess the necessary tensile strength to be practical in usage and to utilize a reinforcing substance foreign to the substance of which the body of the composition is formed to give to the substance the tensile strength above referred to, and to prevent disintegration of the same.

The invention further consists in the features of construction and combination of parts hereinafter described and claimed.

In the drawings: Figure 1 is a section of a strip of the insulating composition of the present invention; Fig. 2 a face view showing the fire and water proof coating for the composition partially broken away; Fig. 3 a section on an enlarged scale showing the substance in the initial stage of manufacture; and Fig. 4 a view similar to Fig. 3 showing the condition of the substance when completed.

In the construction of steel cars and similar structures, it has been found necessary to pack the walls with some sort of heat and cold insulating substance. The principal object of the present invention is to make such a substance out of vegetable fiber, as for instance shredded hemp, thus producing a substance which is cheap and simple of manufacture, and of a commercial practicability in this particular field. Ordinarily a substance entirely composed of vegetable fibers, as for instance hemp, would not be practicable because of the fact that it would not have the necessary tensile strength and cohesive properties to maintain

it in a compact mass during usage; that is to say, if it were used in the walls of a car the constant vibration imparted to the car body would pound the substance to such an extent as to disintegrate it, thus causing it to lose its compact formation and rendering it inefficient as an insulation. It is therefore necessary in order to practically adapt a substance made of vegetable fibers to this particular usage to reinforce the same in some manner so as to give it the tensile strength and property of cohesion necessary to withstand the jolting and vibration it will be subjected to in use.

It is the aim and object of the present invention to produce a substance which will be practicable as a car insulating substance and eliminate the above noted objections to the use for this purpose of a substance composed mainly of vegetable fibers.

Referring to the drawings, and particularly to Fig. 1 the substance is composed of a mass of vegetable fibers 5, as for instance hemp, and these fibers are pricked or woven through a strip of burlap or other open weave fabric 6. The fabric is preferably placed at approximately the center of the substance as indicated in the drawings. By pricking or weaving the vegetable fibers through this fabric it is obvious that the fabric acts as a tensile reinforcement for the substance, and that the ordinary cohesive properties of the fibers are not depended upon to hold the mass together. By utilizing this reinforcing strip the material can be made from vegetable fibers thus rendering its production cheap, and at the same time it will contain the necessary tensile strength to prevent its falling apart or disintegrating in use in the manner heretofore described. If desired a layer of fire and water proof material 7 may be applied to the outer faces of the insulating substance.

In manufacturing this substance the fibers are first pricked or woven through the fabric as indicated in Fig. 3 after which they are subjected to a pressure and formed into a compact mass as indicated in Fig. 4. When subjected to this pressure the fibers will mat together in a manner so as to form a body sufficiently compact to prevent penetration of heat, cold or moisture therethrough, and this combined with the property of tensile strength given to it by the use of the fabric will produce an insulating substance well

adapted for the practical requirements of the purpose intended.

I claim:

As a new article of manufacture, an insulating substance comprising a central strip of open weave fabric and a mass of vegetable fibers pricked through and intermeshed with said fabric, to lie on both sides thereof said fabric and intermeshed fibers

when pressed forming a compact tensile<sup>10</sup> reinforced mass of fibers and a coating of fire and water-proof material on the outside of said mass, substantially as described.

LOWELL C. BASSFORD.

Witnesses:

H. U. MORTON,  
HENRY SANDS.